

## [54] NOVEL DISCHARGE LAMP AND COATING

[75] Inventors: **Ferinand Rokosz**, Clifton; **Joseph W. Sausville**, Glen Rock, both of N.J.

[73] Assignee: **Westinghouse Electric Corporation**, Pittsburgh, Pa.

[22] Filed: **July 3, 1973**

[21] Appl. No.: **376,254**

[52] U.S. Cl..... **313/487**, 117/33.5 L, 252/301.4 R

[51] Int. Cl..... **H01j 1/62**

[58] Field of Search..... 313/109, 108; 252/301.4 R; 117/33.5 L

## [56] References Cited

## UNITED STATES PATENTS

|           |         |                       |             |
|-----------|---------|-----------------------|-------------|
| 2,714,095 | 7/1955  | Kobuke.....           | 252/301.4 R |
| 2,838,705 | 6/1958  | Hierholzer.....       | 313/109     |
| 3,417,027 | 12/1968 | Wanamaker et al.....  | 313/109     |
| 3,571,648 | 3/1971  | Saitama-Ken.....      | 313/109     |
| 3,670,193 | 6/1972  | Thorington et al..... | 313/109     |

Primary Examiner—James W. Lawrence

Assistant Examiner—Harold A. Dixon

Attorney, Agent, or Firm—R. A. Stoltz

## [57] ABSTRACT

A color corrected discharge lamp combination providing an emission with a very desirable color similar to that of an incandescent lamp, but maintaining the efficiency and long life advantages of a discharge lamp. The lamp is similar to a normal high-pressure mercury discharge lamp, but also contains a non-luminescent coating of silica, titania, magnesia or alumina or mixtures thereof on the interior surface of the outer envelope to provide a color-shift and a phosphor coated over the non-luminescent coating. The phosphor mixture substantially comprises 70-90 percent by weight of yttrium vanadate phosphor or yttrium phosphate-vanadate phosphor and 10-30 percent by weight of magnesium fluoro-germanate or magnesium arsenate.

## 2 Claims, 3 Drawing Figures



PATENTED JUL 23 1974

3,825,792

SHEET 1 OF 2



FIG. 1

PATENTED JUL 23 1974

3,825,792

SHEET 2 OF 2



FIG.2



FIG.3

## NOVEL DISCHARGE LAMP AND COATING

## BACKGROUND OF THE INVENTION

This invention relates to high-pressure mercury discharge lamps, and more particularly to discharge lamps having a color similar to that of an incandescent lamp and having good color rendition and high efficiency.

Since the advent of the use of high-pressure mercury discharge lamps for general lighting purposes, it has been apparent that an improvement in quantity of light was gained, but, where the color of objects viewed under the light source was of importance, the quality of the light emitted from such lamps had shortcomings. This was primarily due to the lack of radiation in the red portion of the visible spectrum. As a result, the use of the high-pressure mercury discharge lamp was primarily limited to applications where lamp efficiency was of prime consideration and source color or color rendition from the source were of minor importance, for example, in highway, street and parking lot lighting.

The incandescent lamp, which has abundant emissions in the red portion of the visible spectrum has been in use for a long time and users have become "accustomed to" its radiation. When the high-pressure mercury discharge lamp came into use, users compared it with the incandescent lamp, and it became evident that unless the emission spectrum of the high-pressure mercury lamp was changed, it would never replace incandescent lamps where aesthetics were involved. One method of modifying the spectrum of the high-pressure mercury discharge lamp is to coat the inner surface of the outer envelope with a phosphor. Such color corrected high-pressure mercury discharge lamps are well known in the art.

U.S. Pat. No. 2,748,303 issued to Thorington on May 29, 1956 disclosed the use of magnesium fluorogermanate phosphor (activated with manganese with a valence of 4 plus). Lamps of this type have been widely used and typically provide a correlated color temperature of about 4,100°K Kelvin with a color rendition index of about 43. U.S. Pat. No. 2,615,848 issued to Wells on Oct. 28, 1952 disclosed a high-pressure mercury lamp using a magnesium arsenate phosphor (also activated with manganese with a valence of 4 plus). The magnesium arsenate lamps provide light of a quality similar to that of the magnesium fluorogermanate coated lamps. U.S. Pat. No. 3,569,762 issued to Levine et al on Mar. 9, 1971 discloses a high-pressure mercury discharge lamp with an yttrium vanadate phosphor (activated with europium with a valence of 3 plus). Such lamps typically have a correlated color temperature of about 3,600°K and a color rendering index of about 47. U.S. Pat. No. 3,661,791 issued to Ropp on May 9, 1972 discloses a method for preparing yttrium phosphate-vanadate phosphor (activated with trivalent europium) to be used with a high-pressure mercury discharge lamp. Lamps using such a phosphor have emissions similar to that of lamps using yttrium vanadate.

The internationally accepted method for standardizing and measuring the color rendering properties of light sources is set forth in the publication of the International Commission on Illumination, identified as publication C.I.E. No. 13 (E-1.3.2) 1965.

The radiation from an incandescent filament is well known. The emission is dependent upon the tempera-

ture at which the filament is operated and the locus of emissions for different temperatures as plotted on an ICI color diagram is commonly referred to as "the black body line." In order to maintain a reasonable life of an incandescent bulb, such are generally run at less than 3,100°K and typically at about 2,900°K.

The ICI color system is described in detail in the "Handbook of Colorimetry," by Arthur C. Hardy, The Technology Press, Massachusetts Institute of Technology (1936).

Not only were color corrected mercury discharge lamps of the prior art of too high a correlated color temperature (too blue), but the emission of such lamps was also away from the black body line (the magnesium fluorogermanate lamp, for example, was too green) and therefore inherently provided relatively poor color rendition.

One method which has been used to lower the correlated color temperature is to use a very thick coating of phosphor. Using such a thick coating of yttrium vanadate phosphor, for example, has reduced the correlated color temperature from approximately 3,600° to approximately 3,440°K. Unfortunately, this not only reduces the color rendering index slightly but also dramatically reduces the efficiency.

Silica layers have been used in high pressure mercury vapor lamps. In U.S. Pat. No. 2,838,705, issued to Hierholzer et al. on June 10, 1958 a silica layer is used between the phosphor and a silverized reflector to prevent chemical reactions between the phosphor and the reflector. Silica has also been mixed with phosphors. In U.S. Pat. No. 2,806,968 issued to Thorington on Sept. 17, 1957, silica is mixed with the phosphor, such that less phosphor is required and the cost of the lamp reduced (silica being less expensive than the phosphor).

Apparently none of the lamps of the prior art succeeded in reducing the color temperature to the range of 2,800°-3,100°K while simultaneously holding chromaticity to the black body line and thus none of the lamps achieved an emission of a color similar to that of an incandescent lamp.

## SUMMARY OF THE INVENTION

It has been discovered that a color corrected high-pressure mercury discharge lamp combination with an emission having a color very similar to that of an incandescent lamp, but with the efficiency and long life of a discharge lamp can be obtained using non-luminescent oxide coating of silica, magnesia, titania or alumina (or mixtures thereof) on the interior surface of the outer envelope with one of certain phosphor mixtures coated over the non-luminescent oxide coating. The phosphor mixtures use a manganese-activated phosphor and a europium-activated phosphor, the manganese-activated phosphor being at least one of magnesium fluorogermanate and magnesium arsenate, and the europium-activated phosphor being at least one of yttrium phosphate vanadate and yttrium vanadate. The mixture uses about 83 percent by weight of europium-activated phosphor to 17 percent by weight of manganese-activated phosphor. The combination achieves a correlated color temperature of about 3,000°K with a color rendering index of about 60.

In particular, it has been discovered that principally submicron particles of the above mentioned non-luminescent oxides provide a color shift which could

not be obtained by varying the percentages in the phosphor blend and this color shift, together with certain phosphor blends, makes possible an incandescent-color high pressure mercury discharge lamp.

#### BRIEF DESCRIPTION OF THE DRAWINGS

For a better understanding of the invention, reference may be had to the exemplary embodiment shown in the accompanying drawings in which:

FIG. 1 is a side elevational view of a discharge lamp constructed in accordance with the present invention, with part of the outer envelope and arc tube broken away;

FIG. 2 illustrates the x,y-chromaticity diagram of the ICI system showing the x,y coordinance of the emissions of various lamps; and

FIG. 3 shows the emission spectrum of the lamp of the instant invention, with relative energy plotted against wavelength in nanometers.

#### DESCRIPTION OF THE PREFERRED EMBODIMENT

In FIG. 1 there is shown the general arrangement of a high-pressure mercury discharge lamp within which the non-luminescent oxide coating and the phosphor mixture coating of the present invention are utilized. The lamp, generally designated 10, includes an outer light-transmitting envelope 12 which is sealed to a standard mogul base 14. Mounted within the outer envelope 12 and spaced therefrom is an arc tube 16. The arc tube 16 is mounted within the outer envelope 12 by conventional frame 18 and a pair of straps 20. Sealed within the arc tube 16 disposed at opposite ends thereof is a pair of tungsten operating electrodes 22 and 24. The electrodes 22 and 24 are sealed to opposite ends of the arc tube 16 by a conventional ribbon seal 26. A starting electrode 28 is also sealed to the arc tube adjacent to electrode 24 by means of ribbon seal 26.

The frame 18 is carried by one of a pair of conventional lead-in conductors 30 which extend through a conventional reentrance stem press 32 connected to mogul base 14, which in turn is connected to a conventional power source 34 in the well-known manner. The electrodes 22, 24 and 28 are electrically connected to one or the other of the lead-in conductors 30. A starting resistor 36 is connected between one of the lead-in conductors 30 and the starting electrode 28 to the frame 18.

A charge of mercury 38 is contained within the arc tube 16 and this predetermined amount of mercury will, when fully vaporized during normal operation of the lamp provide a predetermined pressure therein. The arc tube also contains a small charge of an inert ionizable starting gas.

The non-luminescent oxide coating 40 is disposed directly on the interior surface of the outer envelope 12. The phosphor mixture 42 is coated over the non-luminescent oxide coating 40 and thus the two layers are provided with the phosphor-mixture layer 42 being on the inside closer to the arc tube and the non-luminescent oxide layer being on the outside and directly on the interior surface of the outer envelope.

The lamp configuration, (other than the non-luminescent oxide and particular phosphor coatings) is essentially conventional and a more detailed description of its operation may be found in the aforementioned U.S. Pat. No. 2,748,303.

Generally, the non-luminescent oxide coating 40 will be from about 0.2 to 2 milligrams (mg) per square centimeter (and typically about 0.5-0.9 mg per square centimeter). Generally, the coating of the phosphor mixture 42 will be from about 1-8 mg of phosphor per square centimeter of coated area (and preferably about 2.4-2.8 mg per square centimeter).

The particle size of the non-luminescent oxide coating 42 must be principally of submicron size (it must be principally comprised of particles having an average diameter of less than one micron). It has been found, for example, that silica particles having a 0.025 micron average size (such as Pittsburgh Plate Glass's "HiSil") provide a satisfactory coating. It has been found that the particle size is critical and experiments with, for example, titania of a particle size generally greater than 2 microns showed that the desired color shift was not obtained.

FIG. 2 shows the relative emissions of various lamps 20 and also the black body line. Point A represents the emission of a clear (without any phosphor coating) high-pressure mercury lamp. Point B represents the emission of a magnesium fluorogermanate lamp with a normal thickness of phosphor coating. Point C represents the emission of a yttrium phosphate-vanadate lamp. Point D represents the emission of the lamp of the instant invention and Point E represents the emission of a typical incandescent lamp. The line FG is the black body line. The filament temperatures for various points along the black body line are as indicated. As noted previously, the emission of the magnesium arsenate lamp is similar to that of the magnesium fluorogermanate lamp and the emission of the yttrium vanadate is similar to that of the yttrium phosphate-vanadate lamp.

Emissions along the line AC can be obtained by using thinner layers of yttrium vanadate phosphor, and emissions along the line AB can be obtained by using thinner coatings of a vanadate phosphor. Emissions along the line BC can be obtained by a normal coating thickness with a mixture of vanadate and fluorogermanate phosphors. Similarly, points in the triangle ABC can be achieved by thinner layers of mixtures of these phosphors. Points beyond B along the extension of line AB could be obtained by a thicker coating of vanadate phosphor, but such thick coatings severely reduce luminescent efficiency and, because of the cost of the phosphors, significantly raise the cost of the lamp. Surprisingly, an approximately normal thickness of an appropriate mixture of phosphor produces an emission, not inside triangle ABC, but at point D when the appropriate layer of non-luminescent oxide is included.

The relatively inexpensive layer of non-luminescent oxide such as silica deposited on the interior surface of the outer envelope (between the phosphor mixture and the outer envelope) provides a significant shift in the color of the emission. An emission with a color temperature of about 3,000°K in close proximity to the black body line can be obtained using normal phosphor thicknesses. When a proper blend (about 70-90 percent by weight of either yttrium phosphate-vanadate or yttrium vanadate or mixtures of the two) is blended with about 10-30 percent by weight of either magnesium fluorogermanate or magnesium arsenate or mixtures of these two) is placed over a layer of appropriate non-luminescent oxide previously deposited on the inside surface of the light-transmitting outer envelope of a

400 watt high-pressure mercury discharge lamp, the result is a lamp emitting approximately 19,500-20,000 lumens after 100 hours of burning with a source chromaticity of an incandescent lamp. It was found that mixing the non-luminescent oxide with the phosphors into a single layer coating did not produce the desired color shift but that the deposition of the non-luminescent oxide and phosphors in separate layers provided a color shift (for all light leaving the lamp) and the desired color shift was obtained.

A coating of silica can be done, for example, by mixing approximately 39 grams of submicron size silica, together with 170 milliliters of nitrocellulose lacquer and 85 milliliters of butylacetate solvent. This slurry is milled for about 3½ hours and then coated on the bulb. The bulb is then lehred to remove the lacquer binder. After lehring of the silica coating, the phosphor mixture is applied. A first slurry is prepared by mixing 1,200 grams of yttrium phosphate-vanadate or yttrium vanadate phosphor (preferably yttrium phosphate-vanadate) with 775 milliliters of butylacetate solvent and 825 milliliters of nitrocellulose lacquer. A second slurry is prepared by mixing 1,200 grams of magnesium fluorogermanate or magnesium arsenate (preferably magnesium fluorogermanate) with 1,475 milliliters of nitrocellulose lacquer and 600 milliliters of butylacetate solvent. After milling, two slurries can be mixed together to a ratio of 1 part by volume of magnesium fluorogermanate to 4 parts of yttrium phosphate-vanadate and coated on the bulb. The coated bulb is then lehred again to remove the binder. The phosphor mixture which results from this coating process is the preferred mixture and consists essentially of about 17 percent by weight yttrium phosphate-vanadate and about 83 percent by weight of magnesium fluorogermanate.

Magnesia, titania and alumina or mixtures thereof can be substituted in whole or in part for the silica in the preceding examples in approximately the same proportions. Alumina is especially convenient as it does not readily absorb moisture (as compared to magnesia or silica) and is readily obtained in submicron size particles (as compared to titania which is generally available only in particle sizes too large for this application).

FIG. 3 illustrates the emission spectrum of a lamp of the instant invention. Such a lamp has enough emission in the 600-700 manometer region to provide enough red to give an incandescent color, but has very little emission in the infrared region (above approximately

700 manometers). Conversely, the incandescent lamp emits most of its energy in the infrared region, and this energy is generally wasted (and any attempt to get more of the energy in the visible region by raising the filament temperature will, of course, result in further shortening the already relatively short life of the incandescent lamp). Thus, the lamp of the instant invention provides the color of the incandescent lamp, without the low efficiency and short life of the incandescent lamp.

Since numerous changes may be made in the above described high-pressure mercury discharge lamp with its prescribed non-luminescent oxide and phosphor mixture coatings, and different embodiments of the invention may be made without departing from the spirit thereof, it is intended that all matter contained in the foregoing description or shown in the accompanying drawings be interpreted as illustrative and not in a limiting sense.

What is claimed is:

1. In combination with a discharge lamp comprising an elongated light-transmitting arc tube containing a predetermined amount of mercury which when fully vaporized during normal operation of said lamp will provide a predetermined pressure of mercury vapor therein, and an outer light-transmitting envelope having an interior surface spaced from and enclosing said arc tube, the improvement which comprises:

a. a coating of principally submicron particles of at least one non-luminescent oxide selected from the group consisting of silica, magnesia, titania, and alumina disposed directly on said interior surface of said outer envelope; and

b. a phosphor mixture disposed on said non-luminescent oxide coating, said phosphor mixture substantially comprising:

I 70-90 percent by weight of at least one phosphor selected from the group consisting of yttrium phosphate-vanadate activated by europium and yttrium vanadate activated by europium; and

II 10-30 percent by weight of at least one phosphor selected from the group consisting of magnesium fluorogermanate activated with manganese and magnesium arsenate activated with manganese.

2. The combination of claim 1, wherein said phosphor mixture consists essentially of about 83 percent by weight yttrium phosphate-vanadate activated by europium and about 17 percent by weight of magnesium fluorogermanate activated with manganese.

\* \* \* \* \*

UNITED STATES PATENT OFFICE  
CERTIFICATE OF CORRECTION

Patent No. 3,825,792 Dated July 23, 1974

Inventor(s) Ferdinand Rokosz and Joseph W. Sausville

It is certified that error appears in the above-identified patent and that said Letters Patent are hereby corrected as shown below:

On the cover sheet of the patent, the inventors name should be changed from "Ferinand" to --Ferdinand--.

Signed and sealed this 29th day of October 1974.

(SEAL)  
Attest:

McCOY M. GIBSON JR.  
Attesting Officer

C. MARSHALL DANN  
Commissioner of Patents